

April 1, 1930.

P. GREFFIN

1,752,298

PRINTING DIE

Filed April 6, 1927



FIG. 1



FIG. 2



FIG. 3



FIG. 4



FIG. 5

Inventor  
PHILIP GREFFIN

By Paul, Paul Moore

ATTORNEYS

## UNITED STATES PATENT OFFICE

PHILIPP GREFFIN, OF MINNEAPOLIS, MINNESOTA, ASSIGNOR TO MELONE-BOVEY LUMBER CO., OF MINNEAPOLIS, MINNESOTA, A CORPORATION OF MINNESOTA

## PRINTING DIE

Application filed April 6, 1927. Serial No. 181,450.

This invention relates to the art of embossing and printing, and particularly relates to that section of embossing art concerned with pressure work through sheet material, with male and female dies engaging the sheet from opposite sides. The invention is based on the discovery of a new use of a known material, principally for the purpose of producing what is known in the embossing art as the male die. However, the invention is not considered to be limited to the production of male dies, since the material possesses qualities permitting of use in any work where it is the object to compress certain portions of the material and cause other portions to be raised, to provide a printing plate or die. It is to be understood that no claim is made for the production of the material but only to the discovery of a new property in the material by which it may be used for the above mentioned purposes.

The main object of the invention is to provide a material which, when acted on by a die, will receive and retain an impression in relief, in which the raised portions are of sufficient and of equal height to produce what is known in the embossing art as the male die, and to produce such a die having sufficient rigidity to withstand the unusual and prolonged friction and compression strains well known in this art, and yet to provide a die having those qualities which enable it to also act as a cushion.

In order to clearly show the economic value of the discovery of the properties of the herein described material, as a medium for the taking of embossed designs, a presentation of the method now in general use, is given. In the old process some sort of binder board or other suitable material was used as a base for the male die, and this base was overlaid with sheets of paper superposed one after the other to build up the design upon the base. Thus in the original process, the operation was mainly that of building up. This operation was performed in the following manner: A metal or female die was prepared having the desired design. The next step was to form the male die. For this purpose, a base was selected and upon this base was

first secured a piece of paper of sufficient thickness and yieldability to take an embossed impression. An impression was then given to this paper by the metal die, as the result of which a slightly raised design was produced in the paper. Another sheet of paper was then laid over and secured to the first, and another impression given, and this process was continued until the high parts of the design had been built up to the desired degree, thus producing the male die with the raised design. This was a very expensive, time-consuming process.

It will be seen that the difficulty encountered in this work is to produce raised portions of sufficient height and to have all raised portions of proper height. In addition it has been difficult to find a material upon which such raised portions could at all be evenly produced, and in which the raised portions were rigid enough to withstand the hard usage to which the die is put. It will be understood that the operation of building up and re-impressing is very time-consuming and expensive and it is the object of this invention to eliminate the necessity for these operations.

To further show the economic value of my discovery a kind of history of my own experiments is given. As above stated, originally book binder board was used. This board is composed generally of fibrous woody material such as wood pulp. The attempt was made to produce the raised or embossed portions by a single, prolonged impression from a metal die. It is evident that if such a thing could be done, the building up operation could be entirely dispensed with. However, in all the materials experimented with except the one described herein, raised portions of proper definition and height could not be produced except by building up in the manner above mentioned.

Attempts were made to form the die in another manner, to-wit: by making the impression in plastic material held upon a suitable base, for example both cement and sealing wax were used. When using these substances, a suitable base was provided and was over-laid with a coat or layer of the sub-

stance, and the impression was made while in a plastic state. However, in these cases it was practically impossible to obtain an even spread, that is one having equal thickness at all portions. Moreover, in both cases the coating would crack under the ordinary working pressures. Thus the objections were, poor definition in the embossed areas, and fracture of the die under pressure. More success was had with cement in regard to the evenness of the "spread," but the substance was too brittle to withstand pressure. Moreover, although the bases were generally formed of compressible material, this did not prevent cracking of the surface coating.

Experiments were made with another material called bakelite. Sheets of this material were used having a thickness of about one-sixteenth of an inch. However, this substance was of such density that sufficient clearly defined embossed areas could not be obtained. Moreover, the embossed portions were of uneven height. This material, also, broke down under pressure, so that a very small number of impressions could be made before the die was rendered useless. The length of life of the die could not be depended on as evidenced by the fact that one might only obtain from five to six impressions. There was always the uncertainty as to whether the die would last until the "run" was completed. Therefore, with using the above materials, it was practically impossible to obtain clear definition and when some degree of uniformity or clarity was obtained, the substance would crack under pressure.

Various so-called builder board materials were also tried but all were brittle and acted under the ordinary working pressures, something in the manner of dry lime, that is, they crumbled. The results were fracture, lack of clean definition and lack of sufficient height of the embossed areas, and uniformity of design, as well as failure to retain the impression.

Another board was tried which is also a pulp board but the materials are ground and the fibre did not have sufficient tensile strength and was too short and thus the material was not sufficiently tough to stand up. It must be understood that toughness combined with compressibility is required, as well as even texture.

The material which I have discovered to be particularly suitable for manufacture of dies is that produced by the explosion of wood fibre and the exploded wood fibre being matted together generally in the manner of the builders boards, but the texture being entirely different, and different to such an extent that the present material is the only one known to me which will unfailingly give clearly defined embossed designs of even height and sufficient rigidity, as a result of a single impression without building up. Moreover, the

material is of even texture and can be successfully carved, that is, without splitting and chipping and without unduly dulling the tools.

A material for use as a male die for the purpose mentioned above must have a medium length, strong fibre which is sufficiently long to make the material tough and to cause it to hold together when being cut. After a large number of experiments it appears that the material must also have a long fine fibre well interwoven in the manner of a felt. Felt itself, however, is too soft, and does not possess sufficient rigidity, nor will such material retain the impression.

The material which I have found to be the best is made from yellow pine in the following manner: Edgings from yellow pine saw mills containing live material and no bark, is cut into blocks approximately two inches square. These blocks or chips are then loaded into what is known as a gun, and are submitted to a steam pressure of about twelve hundred pounds. The steam carries off some of the resinous material but leaves sufficient of natural resinous wood binder to obtain a tough comparatively soft and compressible material which can be cut without breaking or cracking. Thus the natural binding quality of the wood is taken advantage of and sufficient resinous matter is provided so that each fibre is coated with such binder. After the chips have been submitted to the pressure above mentioned, the gun is shot to release and explode the moistened material producing the fine fibre resembling fine cut tobacco. This material is then heated and compressed to form the sheet material, having substantially the properties above described.

The drawings illustrate the method of making the male die, and this illustration is only suggestive of the use of the present material for the purpose of making dies or plates for use in the embossing and printing arts.

Figure 1 is an edge view of a sheet of material from which, in this instance, a male embossing die is to be constructed;

Figure 2 shows the female die making an impression in the newly discovered material. This being the first step in the preparation of the die;

Figure 3 is an enlarged view of the die after the impression, represented in Figure 2, and shows the coating of hardening material placed on the die after impression;

Figure 4 is similar to Figure 3 but shows the addition of a sheet of paper over-lying and adhesively secured to the hardening coat. This figure represents the completed male die; and

Figure 5 illustrates the operation of the press showing the male and female die cooperating to produce an embossed design upon a sheet of material.

The numeral 1 indicates a sheet of the mate-

rial herein described, or material having similar qualities. The numeral 2 indicates a metal die, in embossing work designated the female die, produced in any suitable manner. This die is suitably mounted so that pressure can be applied. Figure 2 shows the first operation which is to make an impression on the material to form the male die. Figure 3 shows the die after being impressed by the metal die 2, and the numeral 3 designates a brushed-on layer of hardening material, such as varnish applied directly to the impressed and embossed surface, and to better enable the raised or embossed portions to stand up under use. It will be noted that with the material having the qualities set forth herein, uniformity of design can be produced, by a single impression. It will be further noted that heights exactly corresponding to those of the metal die are produced, and that, therefore, no building up of the raised portions or any of the impressed part is necessary. It will be further understood that in a given design some parts are given a greater embossed height to accentuate those parts. It has been found that all of these results may be obtained by a single impression.

Figure 4 shows the completed die in which further reinforcement is provided by means of a sheet of ordinary wrapping paper 4. This sheet is adhesively held by and to the coated surface, and in addition to reinforcing the embossed portions, it prevents possible contact between the sheet to be embossed, and the hardening layer. It will thus be seen that as the result of few simple operations, the main one of which is a pressure operation, a male die or impression plate is produced in which proper heights in embossed areas are had, and in which the embossed portions are reinforced to withstand the unusual pressures of the modern presses. The pressure applied is about twenty tons and the length of the impression from two to three seconds. On the old presses, the pressure was substantially instantaneous, and it was found that with the substances like builders board, cement or bakelite that the proper impressions were seldom, if ever, produced. It has further been found that if the pressing operation is continued, as in the modern type of press, that the same difficulty is encountered, that is uniform embossed designs of the proper height are not produced without subsequent impressions and building up with paper or other suitable material. With the material herein described every portion of the design is produced in a clean, well defined manner, and well raised embossed effects are always forthcoming. The material is very cheap, but the cheapness of material is a small item as compared with the time saved on the building-up operation above mentioned.

Figure 5 shows the operation of producing an embossed design on a sheet of suitable ma-

terial indicated at 6. Preliminary to this operation a sheet of oil paper 5 is laid over the sheet 4 as an additional measure to prevent the soiling of the sheet 6 which is to be embossed.

It will be understood from the description that the properties discovered in the material described, as the result of which the material will take the impressions in the manner above set forth, form the main features of my invention. It will be understood, however, that I believe myself to be the first to form a die of the character described which is composed of a single thickness of fibrous material of homogeneous consistency and having a comparatively long well matted together fibre. Some of the known and essential properties necessary for the use set forth herein are: sufficient length of fibre, a natural resinous binder, combined with a certain density arrived at by compressing the material to a predetermined extent. Moreover, I believe myself the first to make a die of the character described composed of a single thickness of matted, compressed cellulose material, the fibres of which are tough and of medium length. Moreover, evenness of texture is necessary.

Furthermore it is to be understood that by using the material having substantially the qualities herein set forth, much wear and tear on the press is avoided, because no building up operation is necessary. It will be further understood that in the building up operation, as when paper is used and as before mentioned, the original impression having been made and a sheet of material having been laid thereon, a number of successive pressure movements were necessary in order to depress certain portions and raise other portions of the over-laid sheet of paper. It was necessary to make these impressions several times for each overlay. Thus it can be seen what a great saving is made both in the matter of time and in the wear on the press, by being able to obtain a die with a single impression.

I claim as my invention:

1. A die constructed from a material composed of exploded and matted together wood fibre.
2. A die constructed from a material composed of exploded and matted together pine wood fibre.
3. A die constructed from a material composed of exploded and matted together live yellow pine fibre.
4. A die constructed from a material composed of exploded and matted together wood fibre, the fibre being comparatively long and tough and containing a large proportion of its natural resinous matter.
5. A die constructed from a material composed of exploded and matted together yellow pine wood fibre, the fibre being compara-

tively long and tough and containing a large proportion of its natural resinous matter.

5 6. A die constructed from a material comprising yellow pine fibre in which the fibres have been exploded and matted together and in which the fibres contain natural resinous material as a binder, the said material after explosion having been heated and compressed.

10 7. A die constructed from a material comprising live pine fibre in which the fibres have been exploded and matted together and in which the fibres contain natural resinous material as a binder, the said material after explosion having been heated and compressed.

15 8. A die constructed from a yieldable material and comprising a tough wood fibre matted together.

20 9. A die constructed from compressible material comprising wood fibre in which the fibres have been exploded and matted together, and in which the fibres retain the natural resinous material as a binder.

25 10. A die constructed from a compressible material consisting of relatively tough fibre matted together and in which the fibres retain natural resinous material as a binder, the said material having been heated and compressed to form a sheet.

30 11. A die constructed from a yieldable material and composed of a tough, comparatively long wood fibre matted together.

35 12. A die having a base composed of a single thickness of fibrous material, said die having an embossed surface, and having a coating of varnish-like material over this embossed surface, and further having a sheet of paper over-lying and adhesively held by the varnish-like coating.

40 13. A die having a base composed of a single thickness of fibrous material of homogeneous consistency, said die having an embossed surface, and having a coating of varnish-like material over this embossed surface and further having a sheet of paper over-lying and adhesively held by the varnish-like coating.

45 In witness whereof, I have hereunto set my hand this 29th day of March, 1927.

PHILIPP GREFFIN.